

## UNITED STATES PATENT OFFICE

WILLIAM M. PHILLIPS, OF BIRMINGHAM, AND GUY M. COLE, OF DETROIT, MICHIGAN,  
ASSIGNORS TO GENERAL MOTORS CORPORATION, OF DETROIT, MICHIGAN, A COR-  
PORATION OF DELAWARE

## COATING SURFACES OF IRON OR STEEL

No Drawing.

Application filed January 26, 1929. Serial No. 335,384.

The invention relates to the formation of protective coatings upon articles having surfaces of iron or steel and, more particularly, to the deposition of such coatings by electrolytic or partially electrolytic methods. To this end the invention contemplates the exposure of the surfaces in an electrolytic bath in which the article is made the cathode, the bath being of such composition that an insoluble phosphatic coating is formed directly upon the surfaces.

The bath used is one containing a phosphate or phosphates, preferably of zinc, together with a small amount of free phosphoric acid. It may be prepared in various ways and with considerable variation in composition, the following being given as typical examples.

In preparing the bath a zinc oxide may be dissolved in phosphoric acid to form a phosphate or phosphates of zinc, an excess of acid being preferably used in forming the solution, which excess is afterward neutralized to a certain point by addition of an alkali, for example, sodium hydroxide or carbonate. In following this procedure, a considerable range of concentration is permissible, deposits of satisfactory character having been obtained with solutions made with from one to fifteen grams of zinc oxide per liter of bath. The following is suggested as desirable: For one liter of bath, dissolve 5 grams of  $ZnO$  in 23 c. c. of syrupy (about 85%)  $H_3PO_4$ , neutralizing the excess of acid, after solution is completed, by addition of  $NaOH$  until a white precipitate just begins to form. This leaves in the bath a very slight excess of phosphoric acid.

With this bath maintained at near the boiling temperature, with a steel anode and the steel article to be coated connected as cathode, supplying current at a current density at the cathode of 10-15 amperes per square foot, a dense black coating of phosphate or phosphates is obtained on the cathode in a very few minutes.

Other compounds may be employed in preparing the bath, in forming a phosphate or phosphates of zinc as in the above illustration, provided the compound used does not

introduce an anion which would interfere with the formation of the phosphatic coating. Zinc carbonate, for example, might be used in place of zinc oxide.

The bath may also be prepared by dissolving in water other phosphates of zinc, for example, the acid zinc phosphate,  $Zn(H_2PO_4)_2$ , which, as is well known, may be obtained by dissolving metallic zinc in concentrated orthophosphoric acid. The concentration suggested is from 5 to 8% of phosphate. The required quantity of free acid can be added to maintain the acidic character of the bath.

The content of free phosphoric acid should be controlled within relatively close limits. The amount which we have found desirable is in the neighborhood of 0.05 to 0.13%. An excessive content of free acid is likely to result in the deposition of more metallic zinc in the coating, whereas, with the proper acid content, the black phosphatic coating alone is obtained.

The current density also affects the character of the deposit. An increase of current density tends to cause deposition of free metallic zinc along with the black phosphatic coating, so that control of the current density is necessary if the latter coating only is desired. The presence of metallic zinc is not at all detrimental if the coated surface is not to be further treated, or if the further treatment is to consist merely in applying a coating of oil or the like. If, however, the article is to receive a finish of such coating material as paint, lacquer or enamel, it is desirable that no free metallic zinc should be present on the surface to be so coated.

In treating the surface for reception of such finishes as paint, lacquer or enamel, the treatment should be such as to leave on the exposed surface only the phosphatic coating. Should the control of acidity and current density not be such as to avoid the deposition of zinc, the free zinc may be converted into the phosphatic coating by mere exposure to the bath without passage of current. A reaction takes place between the zinc and the constituents of the bath affected possibly by the presence of iron, resulting in the forma-

55

60

65

70

75

80

85

90

95

100

tion of the coating of insoluble phosphate or phosphates on the exposed surfaces. It may be desirable, in some cases, to supply the current intermittently, thus providing intervals during which the reaction may proceed between the electro-deposited zinc and the ingredients of the bath.

While a steel anode is regarded as preferable, it is not considered essential, as zinc, for example, has been used. The voltage varies with the concentration of the constituents of the bath. From one to six volts have been found satisfactory. The bath should be maintained at a high temperature, near the boiling point being considered desirable.

The coating of phosphatic character produced by our process is of a deep black color and adheres closely to the iron or steel surfaces. It is found to impart very high resistance to rust-producing agencies and also affords an excellent foundation for reception of other coatings such as oil, paint, lacquer or enamel with greatly increased effective life of the finish.

26 Variations may be made from the exact details above set forth, and therefore the invention should not be understood as being restricted to such specific disclosure except as required by the terms of the appended claims.

30 We claim:

1. The process of treating articles having surfaces of iron or steel comprising exposing such surfaces in a bath containing a solution of zinc phosphate, and passing current through the bath and the article as cathode to effect an electrolytic deposition of zinc upon such surfaces.

2. The process of treating articles having surfaces of iron or steel to produce thereon a phosphatic protective coating comprising exposing the surfaces to the action of a bath containing a salt from which zinc may be electrolytically deposited upon said surfaces and phosphoric acid compound adapted to react with such deposit to produce such protective coating, and passing current through such bath and article to effect deposit of zinc on said surfaces.

3. The process of treating articles having surfaces of iron or steel to produce thereon a protective coating comprising electrolytically depositing zinc upon said surfaces and simultaneously exposing said zinc deposit to the action of phosphoric acid compounds effective to convert such deposit into protective salts containing zinc.

4. The process of forming a zinc-containing protective coating upon articles having iron or steel surfaces comprising exposing such surfaces in a bath containing phosphoric acid and one or more zinc compounds thereof, passing current through the bath and the article as cathode to deposit metallic zinc thereon, interrupting the deposition of zinc and permitting the article to remain in the bath

while reaction takes place between the phosphoric acid compounds thereof and the electrodeposited zinc.

5. The process of forming a phosphatic coating upon articles of ferrous metal comprising exposing the articles to a bath containing a solution of zinc phosphate and free phosphoric acid, the acid being within the approximate limits of 0.05 to 0.13 percent, passing current through the bath and the article as cathode with a voltage sufficient to deposit metallic zinc on the article and continuing the exposure to the bath to cause reaction of the deposited zinc to form zinc phosphate on the surface.

6. A ferrous metal article coated with a mixture of metallic zinc and zinc phosphate.

In testimony whereof we affix our signatures.

WILLIAM M. PHILLIPS.  
GUY M. COLE.

83

90

95

200

105

110

115

120

125

130